

Dec. 4, 1923.

1,476,226

R. A. GRIMOIN-SANSON

## WATERPROOFING PROCESS FOR TEXTILE FABRICS, PAPER, AND SUCH MATERIALS

Filed Nov. 26, 1921



*INVENTOR*

Paul Adrien Grimoin-Sanson

BY *Emil Bounelyte*  
ATTORNEY

## UNITED STATES PATENT OFFICE.

RAOUL ADRIEN GRIMOIN-SANSON, OF OISSEL, FRANCE.

## WATERPROOFING PROCESS FOR TEXTILE FABRICS, PAPER, AND SUCH MATERIALS.

Application filed November 26, 1921. Serial No. 517,926.

*To all whom it may concern:*

Be it known that I, RAOUL ADRIEN GRIMOIN-SANSON, citizen of the Republic of France, and resident of Oissel, France (post-office address Chateau d'Oissel), have invented a new and useful Waterproofing Process for Textile Fabrics, Paper, and Such Materials, which improvements are fully set forth in the following specification.

10 Textile fabric waterproofing processes are already known according to which the rubbered surface to be waterproofed is sprinkled with cork. But the cork penetrates only slightly into the india-rubber, the result being that the coating, while resistant at the surface frequently becomes spoilt or altered inside.

Attempts have been made to remedy this drawback by applying several successive 20 layers or coatings of cork, but it has been found that, after the first application of cork, the cork coating or layer cannot be coated with rubber.

The object of my invention is to provide a 25 waterproofing process, consisting in coating textile fabrics, paper, and such materials, with a number of india-rubber layers successively covered over with a layer or coating of powdered cork, the result being to make the 30 fabric or other material absolutely hot-washable and hot ironable, just like ordinary linen.

To the aforesaid advantages are added 35 great strength, extreme lightness and small cost.

My invention is essentially characterized by a special treatment for and of the cork powder to be sprinkled over the rubber layers or coatings.

40 The cork powder collected in bottle-cork factories is damp and sticky.

According to the process which is the object of my invention and in order to free the said powder from impurities which make 45 it unsuitable for coating, it is soaked for about 24 hours in the following mixture which should previously have been subjected to a careful and thorough mixing:

Water 100 grams.

50 Carbonate of soda 5 grams.

(It should be understood, of course, that the above proportions are given only as an example).

55 After having allowed the powder to soak for 24 hours, it has to be completely dried by

aerating it with air heated up to (say) 60 degrees centigrade.

After complete drying, an operation which requires about two hours, the said powder is screened and is then ready for use.

60 This powder will take as many rubber coatings or layers as desired if, in front of the spreading knife, a roller saturated with benzene is arranged and the following method is practiced:

65 After having put on one or two rubber layers or coatings, according to the fabric to be treated, the cork is applied simply by causing the fabric to pass, when leaving the knife, beneath a hopper mounted on the 70 work-table (about one meter fifty centimeters from the knife) and containing powdered cork prepared as above stated. As the fabric passes beyond the hopper the cork is pressed into the rubber by a pair 75 of coating rolls.

The other coatings are put on as usual, subject to a felt roller saturated with benzene being placed in front of the spreading 80 knife, such roller priming the cork and causing it to adhere tightly to the rubber.

Finally the fabric is thoroughly calendered.

85 One form of apparatus for carrying out the described process is represented in the annexed drawing in diagrammatic side elevation, with parts in section. The component elements of this apparatus are as follows:

A is the roll for receiving the fabric after a single layer of rubber and cork has been applied thereto;

B, the felt roller saturated with benzene for treating the fabric so that a fresh coating of rubber will adhere to the previously applied layer of cork;

C, the tank containing the benzene which discharges slowly therefrom upon the felt roller B;

100 D, a large hard-rubber roller where the rubber, indicated at E, is applied and impregnates the fabric which is stretched mechanically and passes beneath the spreading knife F. The latter regulates the application of the rubber, so that the cork which is contained in the hopper I will adhere to this layer or coating of rubber.

105 On passing beyond the hopper, the fabric coated with the powdered cork travels for a distance of about 2½ meters along the work

table J and reaches the small pressure rolls K which cause the cork to penetrate the still soft and fresh layer so as to form with it a homogeneous unit like reinforced cement, 5 not a mere pulverulent cork layer.

As the coating of rubber and cork continues to dry, it is wound up at L and can thereafter have as many more layers of rubber and cork applied to it as may be desired, according to the degree of waterproofness sought. Four layers are generally sufficient. 10

The operation is completed by a very intense calendering between large pressure rolls. The product can thereafter be washed in hot water and ironed with a hot iron without undergoing any change; and the cork so treated can be readily dyed, and is capable of receiving any desired impression or printing. 15

For clothing, inter alia, impressions and colours can therefore be obtained suggestive of fashionable draperies, Scotch checks, etc.

Obviously, the water-proofing process as above set forth can just as well be used for waterproofing paper, calico, or any other similar stuff, subject to the operation being conducted as above stated.

Having now particularly described and 30 ascertained the nature of my said invention and the manner in which the same is to be performed, I declare that what I claim is:

1. A process of producing waterproof material, comprising soaking powdered cork in an alkaline solution, drying the cork, applying a coating of rubber to a sheet of fibrous

material, and then applying the dried cork powder to the coated surface of the sheet; substantially as described.

2. A process of producing waterproof material, comprising soaking powdered cork in a solution of sodium carbonate, drying the cork, applying a coating of rubber to a sheet of fibrous material, and then applying the dried cork powder to the coated surface of the sheet; substantially as described. 40 45

3. A process of producing waterproof material, comprising soaking powdered cork in an alkaline solution, drying the cork, alternately coating a sheet of fibrous material with rubber and applying the dried cork powder to the coated surface of the sheet, and pressing the powdered cork into the rubber after the application of each layer of cork; substantially as described. 50 55

4. A process of producing waterproof material, comprising soaking powdered cork in a solution of sodium carbonate, drying the cork, alternately coating a sheet of fibrous material with rubber and applying the dried cork powder to the coated surface of the sheet, and pressing the powdered cork into the rubber after the application of each layer of cork; substantially as described. 60 65

In testimony whereof I have signed this specification in the presence of two subscribing witnesses.

RAOUL ADRIEN GRIMOIN-SANSON.

Witnesses:

FERNARD DUFOUR,  
CHARLES LEON LOISEL.